

## UNITED STATES PATENT OFFICE.

WILBUR FRANCIS CRAWFORD, OF WACO, TEXAS.

## WATERPROOFING COMPOSITION AND PROCESS FOR MAKING SAME.

No Drawing.

Application filed November 13, 1924. Serial No. 749,796.

*To all whom it may concern:*

Be it known that I, WILBUR FRANCIS CRAWFORD, a citizen of the United States, residing at Waco, in the county of McLennan and State of Texas, have invented certain new and useful Improvements in Waterproofing Compositions and Processes for Making the Same, of which the following is a specification.

10 This invention relates to a composition for making textile water-proof and mildew-proof and a process for making the same.

It is generally recommended that beeswax be used as a base for more effective 15 water-proofing agents, while paraffine and ceresin have been considered as less effective to provide a water-proofing compound. In the preparation of such water-proofing compound it has been proposed to heat the ingredients at a very low temperature or at 20 such temperature as will be required only to melt the ingredients, and furthermore where gasoline has been employed as a solvent, a very low temperature has been maintained 25 when the gasoline has been added.

It is an object of this invention to provide a water-proof composition which when manufactured, has its basic ingredients such as paraffine and wool grease, maintained at 30 the boiling temperature so that as gasoline, a solvent, is poured into the boiling ingredients, a more intimate and mechanical mixture will be had.

Another object of the invention is the 35 provision of a water-proof and mildew-proof composition which may be readily applied, will not harden or crack, give off any disagreeable odors, will retain its color, and which will not only prevent mildew, but 40 will also prevent any form of bacterial action.

A further object of the invention is the provision of a process in which paraffine wax may be employed in a water-proof 45 compound as effectively as beeswax, and in which the gasoline as a solvent is added to the boiling paraffine with linseed oil and such other coloring matter and body forming ingredients as may be desired.

50 This invention will be best understood from a consideration of the following detailed description; nevertheless, it is to be understood that the invention is not confined to the disclosure, being susceptible of such

changes and modifications which shall define no material departures from the salient features of the invention as expressed in the appended claims.

Experience has shown where water-proof and mildew-proof canvas is manufactured 55 in large quantities and used in a very hot climate, such as Texas, the following ingredients and in the proportions named, such as 200 pounds of paraffine, 10 gallons of boiled linseed oil, 90 pounds of dry yellow ochre, 20 pounds of litharge (lead oxide), 6 pounds of dry burnt sienna, 4 pounds of dry burnt umber, 30 gallons of gasoline, 20 pounds of degras or wool grease will 60 provide a cloth which is pliable, soft, water-proof, mildew-proof and free from bacterial 65 reaction after indefinite exposure.

In carrying out the process, the paraffine and wool grease are heated together in a 70 steam boiler until they come to ebullition.

Linseed oil is placed in a vessel, and the litharge is mixed with the linseed oil and thoroughly stirred until no particles of the litharge are visible. To this composition in the vessel, the burnt sienna, burnt umber and yellow ochre are added, and the whole is stirred until it has become a liquid mass devoid of lumps. This mixture is then poured into the boiling paraffine and wool 75 grease with thorough mixing, and while 80 these ingredients are in the state of ebullition the quantity of gasoline is slowly poured into the same and thoroughly incorporated. The entire composition is then held to boiling point for approximately five 85 minutes.

The liquid mass is maintained at about 100 degrees Fahrenheit, and the material to be water-proofed is saturated by drawing the fabric through the composition placed 90 in a tank, and then the fabric is passed through rollers which press out an excess of the water-proofing. The fabric is dried by 95 causing air to circulate about the same for approximately thirty-six hours although the treated fabric may be applied or used after twelve hours of drying.

It requires approximately 100 gallons of composition to proof 1500 yards of 29 inch, 8 ounce duck or canvas, the quantity varying according to the width, weight, and length of the material.

Paraffine is a wax which is used as a base

and when properly treated will form an absolute water-proofing base, equal in every respect to the well known and expensive beeswax. It is resistant to acid, repellant to water and will thoroughly penetrate canvas when heated to a temperature of 112 degrees Fahrenheit. By the treatment of the paraffine with the other materials, and particularly with the gasoline when the paraffine has been raised to a state of boiling, the fabric material when water-proofed will remain in a soft pliable condition, and will not deteriorate or lose its pliability after prolonged exposure to heat or cold.

15 Degas or wool grease is used for its water repellent properties and to off-set the hardening qualities of the paraffine, thereby making canvas which is water-proofed with the composition more pliable.

20 Boiled linseed oil is employed for not only its water repelling properties, but as a binder for the incorporation of the dry ingredients.

Litharge is used to increase the drying 25 properties of the oils and the yellow ochre as a filler and to aid in the coloring.

Burnt sienna and burnt umber are employed principally for their coloring properties.

30 Gasoline is employed as a solvent and where added to the boiling paraffine and wool grease and the other ingredients causes the ingredients to be thoroughly dissolved and intimately associated in a physical mixture.

35 The ready evaporation of the gasoline acts as a drier for the material.

It must be borne in mind that the gasoline is thoroughly stirred into the mass of boiling ingredients so that the minute particles of the various ingredients have a closer physical association than can be obtained by merely attempting to dissolve them by a solvent when cool.

40 Fabrics so treated are manufactured on a large scale, and experience has shown that such fabrics withstand the intense heat of the State of Texas and other places without deterioration, remain waterproof and do not mildew under unusual circumstances after 50 prolonged exposure.

It is well known that linseed oil has a tendency to injure fabrics, but when so incorporated with the other ingredients in the proper proportions and dissolved while at 55 the boiling point by the gasoline, all danger of the breaking down of the fibers of the fabrics is eliminated.

60 One of the most important advantages flowing from the use of this composition resides in the fact that the article treated is not easily ignited and is therefore fire-resistant to a substantial degree. Also, the extensive commercial use of the invention has demonstrated that the product treated 65 is not susceptible to spontaneous combustion,

as in the case of canvas and the like, treated with other known processes and compositions.

A substantial saving in time is brought about by the use of the herein-described process and composition, since the time for preparation of the composition requires only about one hour, as against twenty-four hours or more required for other processes for the same purpose. Further the composition is applied immediately upon mixing and while still boiling as against a long period of setting required between the mixing and the application of other known compositions for the same purpose.

What I claim is:

1. A water-proofing and mildew-proofing composition comprising 200 pounds paraffine wax, 20 pounds wool grease, 10 gallons of boiled linseed oil, 90 pounds of dry yellow ochre, 20 pounds of litharge (lead oxide), 6 pounds of dry burnt sienna, 4 pounds of dry burnt umber, and 30 gallons of gasoline.

2. A process of forming a water-proofing and mildew-proofing composition which comprises heating paraffine and wool grease to the boiling point, thoroughly mixing linseed oil, litharge, burnt sienna, burnt umber and yellow ochre and adding this mixture to the boiling paraffine and wool grease, then adding gasoline and maintaining the same at the boiling point.

3. A process of forming a water-proofing and mildew-proofing composition which comprises raising paraffine and wool grease to the state of ebullition and separately mixing linseed oil and litharge, adding to the second mixture burnt sienna, burnt umber and yellow ochre, adding this mixture to the boiling paraffine and wool grease and maintaining the whole at the boiling point for approximately five minutes.

4. The herein-described process of forming a waterproofing and mildew proofing composition which consists in mixing paraffine, wool grease, linseed oil, litharge, burnt sienna, burnt umber, yellow ochre and gasoline and bringing all the ingredients, including the gasoline to a boiling point during mixing.

5. The herein-described process of forming a waterproofing and mildew proofing composition which consists in mixing paraffine, wool grease, linseed oil, litharge, burnt sienna, burnt umber, yellow ochre and gasoline and bringing all the ingredients, including the gasoline, to a boiling point during mixing, and maintaining the same at the boiling point during the commingling of the ingredients.

6. A process of forming a waterproofing and mildew proofing composition which comprises raising paraffine and wool grease to the state of ebullition and separately

mixing linseed oil and litharge, adding to the second mixture burnt sienna, burnt umber, and yellow ochre, and adding gasoline during boiling to the mixture.

5 7. A process for forming a water-proofing and mildew-proofing composition for textiles which comprises mixing paraffine wax,

wool grease, linseed oil, coloring matter and gasoline and then bringing all the ingredients, including the gasoline, to the boiling <sup>10</sup> point during mixing.

In testimony whereof, I affix my signature.

WILBUR FRANCIS CRAWFORD.